

Feb. 27, 1940.

R. STEVENS

2,191,810

METHOD OF SENSITIZING PHOTOGRAPHIC SILVER HALIDE EMULSIONS

Original Filed June 28, 1935



NON-SENSITIZED SILVER  
BROMIDE EMULSION

FIG. 1.



SILVER BROMIDE EMULSION  
SENSITIZED WITH 2-2'  
DIMETHYL THIODIAZOL-  
CARBOCYANINE ETHYL  
JODIDE

FIG. 2.



SILVER BROMIDE EMULSION  
SENSITIZED WITH 2-2'  
DIMETHYL-7-METHYL-  
THIODIAZOL CARBOCYANINE  
ETHYL JODIDE

FIG. 3.



SILVER BROMIDE EMULSION  
SENSITIZED WITH 2-2'  
DIMETHYL THIODIAZOL-  
PENTAMETHINE CYANINE  
METHYL JODIDE

FIG. 4.



SILVER BROMIDE EMULSION  
SENSITIZED WITH 2-2'  
DIMETHYL THIODIAZOL-  
HEPTAMETHINE CYANINE  
METHYL JODIDE

FIG. 5.



SILVER BROMIDE EMULSION  
SENSITIZED WITH 2-  
METHYL THIODIAZOL-  
BENZO-CARBOCYANINE  
ETHYL JODIDE

FIG. 6.

INVENTOR  
RENÉ STEVENS

*René Stevens*

ATTYS.

## UNITED STATES PATENT OFFICE

2,191,810

## METHOD OF SENSITIZING PHOTOGRAPHIC SILVER HALIDE EMULSIONS

René Stevens, Antwerp, Belgium, assignor to Gevaert Photo-Producten N. V., Antwerp, Belgium

Original application June 28, 1935, Serial No. 28,870. Divided and this application February 13, 1936, Serial No. 63,737. In Austria July 21, 1934

## 5 Claims.

(Cl. 95—7)

This invention, which constitutes a division of my parent application Ser. No. 28,870 filed June 28, 1935, relates to photographic emulsions sensitized with a new class of dyes, containing in their formula the thiadiazole, oxadiazole or selenodiazole ring



10

wherein X stands for sulphur, oxygen and selenium.

Various salts of heterocyclic bases have hitherto been used for the manufacture of cyanine dyes and styryl derivatives.

In comparison with the known dyes, the new compounds are characterized by a very strong sensitizing power.

Moreover, they show a very high solubility not only in the usual organic solvents, but even in water.

In comparison with the nearest related thiadiazoles, they have a better resistance to acid and are produced with a much higher yield.

These favourable characteristics must be attributed to the special molecular arrangement in which the basic nature of the nitrogen atoms is neutralized by the negative character of the symmetrically placed sulphur atom.

For carrying out the process, the base is prepared according to the methods described by Stollé, Journal für praktische Chemie (2) vol. 69, p. 145-160.

The base is then condensed to an alkyl-quaternary salt, by means of an appropriate ester, for instance: dimethylsulphate, ethyliodide, methyl-iodide or another alkyl ester of Cl, Br, I, SO<sub>4</sub>·CH<sub>3</sub>, ClO<sub>4</sub> or the like. This quaternary ammonium salt is treated in an appropriate solvent as for instance pyridine or acetic anhydride with any known condensing agents, as for instance p-dimethyl amino benzaldehyde, an alkylester of an orthoacid,  $\beta$ -aethoxyacroleinacetal, diphenylformamidin, glutacon aldehyde dianilide hydrochloride and the like.

The following examples illustrate the invention.

## Example I

30 grams of dimethylthiadiazole ethiodide, prepared by heating together on the water bath for half an hour, equimolecular quantities of dimethylthiadiazole and ethyliodide, are dissolved in 200 cc. of acetic anhydride and, after addition of 50 cc. of triethyl ortho-formic acid ester, the whole is boiled together for about an hour.

The dye is precipitated by addition of ether and dissolved in alcohol. A fractional precipitation permits the separation of two dyestuffs. First may be isolated a blue purple dye corresponding most probably with the formula:



10

15

and which sensitizes a silver bromide emulsion nearly uniformly till about 680 $\mu\mu$  with a maximum at 590 $\mu\mu$ .

A further precipitation isolates a yellow orange dye corresponding most probably with the formula:



25

and which sensitizes to about 570 $\mu\mu$  with a very high maximum at about 540 $\mu\mu$ . Either dyestuff may be incorporated in a gelatino-silver bromide emulsion preferably in a concentration of about 0.05% of the silver bromide weight.

## Example II

A mixture of 40 grams of dimethyl thiadiazole ethiodide, prepared by heating together at 100° under pressure 1 mol. of dimethylthiadiazole and 1 mol. of ethyliodide for 24 hours, and 20 grams of dimethylaminobenzaldehyde in 200 cc. of alcohol is heated to boiling. To the boiling solution are added 5 grams of piperidine and boiling is continued for about an hour.

The yellow dye which separates by cooling corresponds most probably with the formula:



50

and sensitizes silver bromide gelatine emulsion with a maximum at about 550 $\mu\mu$ .

55

## Example III

A mixture of 30 grams of dimethyl thiodiazole ethiodide, 50 cc. of triethyl-ortho-acetic acid ester and 250 cc. of pyridine is boiled for about three hours.

After addition of ether, the dyestuff corresponding most probably with the formula:



15 precipitates.

Incorporated in a silver bromide gelatine emulsion, the dye imparts to it a strong sensitivity with a maximum at about 535μμ.

## Example IV

30 grams of dimethyl thiodiazole ethiodide and 50 cc. of β aethoxyacroleinacetal are dissolved in 250 cc. of pyridine and boiled for an hour.

25 The blue dye which can be isolated after addition of ether corresponds most probably with the formula:



35 and sensitizes a silver bromide gelatine emulsion with a maximum at about 650μμ.

## Example V

A solution of 27 grams of dimethyl thiodiazole ethiodide and 50 grams of quinoline ethiodide in 40 500 cc. of absolute alcohol is heated to boiling.

To the boiling solution are added 2.3 grams of sodium dissolved in about 50 cc. of anhydrous alcohol and boiling is continued for about 15 minutes.

45 The dye is separated by precipitation with ether and recrystallized from alcohol.

It corresponds most probably with the formula:



55 and sensitizes a silver chloride gelatine emulsion with a maximum at about 500μμ.

Other symmetrical and unsymmetrical dyestuffs can be obtained for instance by means of 60 the condensation product of dimethyl thiodiazole ethiodide with diphenyl formamidine of the following probable formula:



70 This condensation product can easily be obtained by melting together in an oil bath at 120° one mol. of diphenylformamidine with one mol. of dimethyl thiodiazole ethiodide. The crude product is purified by crystallization from al- 75 cohohol.

## Example VI

A mixture of 25 grams of the above-named condensation product and of 20 grams of quinaldine ethiodide in 250 cc. of pyridine is boiled for two hours. On cooling, the dye corresponding most probably with the formula:



15 separates and is recrystallized from alcohol. It sensitizes an emulsion to 660μμ.

In all the foregoing examples only the dimethyl derivative has been used because of its easy synthesis, so that the dyestuffs produced are methyl derivatives. Other alkyl derivatives, more particularly the ethyl derivatives, are however also useful. It enters therefore into the scope of the invention, that one or both of the CH<sub>3</sub> groups may be exchanged for any suitable reactive group or for instance —CH<sub>2</sub>—CH<sub>3</sub>, —Cl, —S, —SH.

Moreover, the atom of sulphur in the thiodiazole ring may be exchanged for oxygen or sele-

nium.

The substitution of oxygen for sulphur leads to dyestuffs which have an absorption spectrum and a sensitizing action for smaller wave lengths than the corresponding thiodiazole dyestuffs.

The substitution of selenium for sulphur leads to dyestuffs which have an absorption spectrum and a sensitizing action for longer wave lengths than the corresponding thiodiazole dyestuffs.

It is to be understood that the invention is not limited to the foregoing examples or to the specific details given therein.

The drawing affixed to this specification and forming part thereof shows sensitizing curves.

In the drawing:

Fig. 1 is the sensitizing curve of a non-sensitized silver bromide emulsion as usually employed for photographic materials, while

Figs. 2 to 6 show corresponding curves of an emulsion of the same kind when sensitized by an addition of the dyestuffs described in the above Examples 1 and 3 to 6, respectively.

The dye may be added to the emulsion in the form of a solution. It may be incorporated in the emulsion during any stage of its production or the finished emulsion layer may be bathed in a solution of the dye.

I claim:

1. As a photographic material, a silver halide emulsion with an addition of a dyestuff of the general formula



65 wherein R is a member of the group constituted by methyl and ethyl, while Y and Y' are alkyls. "An" is an anion, X is a member of the group constituted by sulphur, oxygen and selenium and Z represents the non-metallic atoms necessary to complete a heterocyclic nucleus selected from the group consisting of five- and six-membered heterocyclic nuclei; n being zero or an integer.

2. As a photographic material, a silver halide emulsion with an addition of a dyestuff as defined

in claim 1, wherein the nucleus, which is completed by the atoms represented by Z, forms part of a condensed system of nuclei.

3. As a photographic material, a silver halide emulsion with an addition of a dyestuff as defined in claim 1, wherein the H of the middle carbon atom of the polymethenyl chain is substituted by an alkyl group.
4. As a photographic material, the silver halide emulsion with an addition of a dyestuff as defined in claim 1, wherein the H of the middle carbon atom of the polymethenyl chain is substituted by the radical

15



20

while  $n=1$ ,  $Y'=Y$  and  $Z$  is



5. As a photographic material a silver halide emulsion with an addition of a dyestuff of the formula



wherein R is a member of the group constituted by methyl and ethyl, while "Hal" is halogen, Y is an alkyl and X is a member of the group constituted by sulphur, oxygen and selenium.

RENE STEVENS. 20